

## UNITED STATES PATENT OFFICE

2,560,514

## PROCESS OF PRODUCING FUR FELT STRIPS

George M. Rickus, Norwalk, Conn., assignor to  
 Hat Corporation of America, Norwalk, Conn.,  
 a corporation of Delaware

No Drawing. Application June 20, 1945,  
 Serial No. 600,651

7 Claims. (Cl. 28—72.3)

**1.** The present invention relates to the formation of fur felt in long strips or yardage by the wool felt process.

As is known in the art, fur felt which has a soft feel and fine texture and appearance and wool felt which has a relatively stiff feel and coarse texture and appearance are made by two distinct processes because of the nature of the fiber. In the fur-felt process, the fur fibers are deposited by suction on a cone larger than the finished size in a relatively thin body which is wet worked and shrunk, as it is felted, into the body of the required size. In the wool-felt process, wool is carded and the web wound on a form into a bat of predetermined thickness and the bat is worked by vibrating pressure means in the presence of steam in a substantially dry process until the bat is compacted to the required thickness.

Fur felt material which is now used in millinery and the like is made by the fur-felt process by depositing fur fibers on very large perforated cones and felting the body, by the usual wet treatment, into a skirt. The skirt is then split into a strip. The formation of these large conical bodies requires longer time and more men to produce than do fur-felt hat bodies so that the output of the equipment is reduced and the cost of making the material is subsequently high.

Efforts to produce fur felt in long strips or yardage by the usual wool-felt process wherein the fibers are carded and a thick bat is formed and mechanically felted to the required thickness have been made. However, they have failed since it was practically impossible to obtain a uniform bat because of the fact that fur, under normal wool-felt conditions, does not card well. The imperfect bats would produce weak and ununiform fabrics which were not satisfactory or acceptable.

Attempts to overcome the failure of the fur to produce a satisfactory bat were made by depositing layers of fur fibers by suction on a belt, a step somewhat similar to the fur-felt process, but these, too, proved unsuccessful in that the bats were not uniform.

The present invention overcomes these difficulties and produces a strip felt in yardage having the handle or feel, texture and appearance of fine 100% fur felt. This is accomplished by preparing with the usual blowing and mixing equipment employed in fur felting, a fur blend and treating the blend so that it will form satisfactory and uniform bats which will felt down on the usual wool-felt equipment into a satisfactory and acceptable fabric.

**2.** I have found that a blend of fur fibers with cotton fibers, treated in accordance with the process set forth in application Serial No. 548-320, filed August 5, 1944, now Patent No. 2,429-073, granted October 14, 1947, to become center-seeking, and hereinafter referred to as center seeking cotton, produces satisfactory felt as do fur fibers blended with a synthetic fiber such as casein, soybean or other protein base fibers (hereinafter referred to as synthetic fibers), and fur fibers blended with said synthetic fibers and center-seeking cotton fibers. Also various types of fur fibers, i. e., fibers of different quality and length, may be blended together to produce a combination of fur fibers satisfactory for use in this process.

The blends including fur fibers and the cotton and/or casein fibers are of particular advantage in that the cotton and/or casein fibers, which replace the short stock in the blend, are relatively long fibers. In other words, the cotton fibers are approximately 1 1/8" long, the casein and soybean fibers are approximately 1 1/2" long and these replace in the blend the short fur fibers which are approximately 1/4 to 1/2" long. These long fibers when mixed with the usual fur fibers which are approximately 3/4 of an inch long produce a blend of relatively long fibers which can be carded and felted in a highly satisfactory and economical manner.

The proportions of fur, synthetic fiber and cotton used in these blends may vary in accordance with the requirements of the fabric. Treated center-seeking cotton gives body, strength and feel to the fabric and also aids in the felting of the fabric. Casein in the blend helps shrinking and aids the felting properties of the blend. Knowing the required properties of the fabric, the proper fibers and the proportions thereof necessary in the blends which will produce a fabric having these properties can readily be determined.

The following blends are not to be considered as defining limitations on the invention but merely examples of the blends that I have used to produce satisfactory felts by the present process. These are: a blend of 60% fur fibers and 40% cotton fibers; a blend of 60% fur fibers and 40% casein fibers; a blend of 60% fur, 20% cotton, 20% casein; a blend of 50% fur, 30% cotton, 20% casein; and a blend of 40% fur, 30% cotton, 30% casein. Each of these felts had the required body, compactness, handle or feel and strength.

**55** I have discovered that the difficulties of carding fur heretofore encountered can be substan-

tially eliminated by treating the blend to insure that the fibers thereof have a proper moisture content. This may be accomplished by humidifying the blend in any suitable manner, such as by storing it preferably at a warm temperature in an atmosphere of between 70 to 80 per cent relative humidity for a period of at least twenty-four hours before it is used.

The blends also may be treated with any suitable emulsion or moistening agent when they are mixed in the fur blending machinery so that they retain the required amount of moisture in the blend.

The treated fur blend is fed to the usual wool carding machine. However, the action of the machine is modified so that it has a less tearing effect on the fibers, which being previously prepared, do not include any noils or the like to be torn apart, and functions primarily as a means for straightening out the fibers into a thin web. One manner of reducing the carding action is by removing some of the carding rollers or reducing the speed of the machine.

The web is fed from the carding machine and formed into an elongate bat of the required thickness and having a predetermined length. I have found it necessary, in order to maintain the blend in proper condition for working during the carding and bat forming operation, to maintain the relative humidity of the atmosphere surrounding the equipment between 70 and 80%.

The bat may be formed in any number of ways. For example, the web from one or more carding machines may be fed to an elongate support, such as a continuous belt, preferably horizontally disposed, to which the end of the web is secured and about which the web is wrapped until the bat of the desired thickness is formed. If necessary, one or more secondary belts or similar means may be disposed adjacent the main belt to engage the bat and hold it against the main belt as it builds up thereon. These secondary belts preferably move synchronously with the main belt and may be yieldably mounted so as to move away from the belt as the bat increased in thickness. After the bat has reached its required thickness it is then cut transversely of the belt and stripped therefrom and then fed to the usual wool hardening machine.

When the bat is formed by bringing together a plurality of webs from different cards and placing them in superposed relation, it may be desired to cause the web from at least one of the cards to be laid back and forth across the other web or webs so that the fibers in one web are crossed by the fibers in the other web. This can be accomplished by feeding in the web at right angles to the main web and laying it back and forth across the main web.

The bat however formed is mechanically hardened by the action of vibrating pressure applying elements in the presence of steam as is usual in the wool felt process.

After the felt strip has been hardened it is fulled with the fulling machinery used in wool felt operations into a fabric. It may then be dyed, preferably by pressure dyeing, to the required color.

After the fabric has been dyed, it is then pounced and finished by any suitable equipment adapted to operate upon yardage goods.

The term "fur" or "fur fiber" used herein

means fur which has been carotted and/or otherwise prepared for felting.

Variations and modifications may be made within the scope of this invention and portions of the improvements may be used without others.

I claim:

1. In the method of producing felt in yardage having the compactness, feel and appearance of fine fur felt, the steps of preparing and moistening a blend consisting of fur fibers and an artificial feltable fiber of the group consisting of center-seeking cotton, casein and soybean fibers, and mixtures thereof; straightening the fibers of the blend into a thin web by a modified carding action and building up an elongate bat from a plurality of thin webs on a support while maintaining the blend in a humid condition; removing the elongate bat from the support; feeding the bat through a hardening machine of the type used in the usual wool felt process to compact and harden the same by vibrating pressure; and fulling the compacted and hardened strip into a fabric.

2. In the method of producing an elongate strip of felt having the texture, feel and appearance of fine fur belt, the steps of preparing and thoroughly intermixing a blend consisting of fur fibers and an artificial feltable fiber of the group consisting of center-seeking cotton, casein and soybean fibers, and mixtures thereof; humidifying the blend; straightening the fibers of the blend into a thin web by a modified carding action; building up from thin webs an elongate bat on a support, maintaining the blend in an atmosphere of 70 to 80% relative humidity during the carding and bat forming; stripping the elongate bat from the support; and hardening and fulling the bat into a fabric by the wool felt process.

3. In the method of producing an elongate strip of felt having the texture, feel and appearance of fine fur felt, the steps of preparing and thoroughly intermixing fur fibers, casein fibers and center-seeking cotton fibers to produce a blend; humidifying the blend; straightening the fibers of the blend into a thin un torn web by a modified carding action; building up from the thin web a thick elongate bat on a support, maintaining the blend humid during the carding and bat forming; removing the elongate bat from the support; and hardening and fulling the bat into a fabric by the usual wool felt process.

4. In the method of producing an elongate strip of felt having the texture, feel and appearance of fine fur felt, the steps of preparing and thoroughly intermixing fur fibers and center-seeking cotton fibers to produce a blend; humidifying the blend; straightening the fibers of the blend into a thin web by a modified carding action; building up from the thin web a thick elongate bat on a support, maintaining the blend humid during the carding and bat forming; removing the elongate bat from the support; and hardening and fulling the bat into a fabric by the wool felt process.

5. In the method of producing an elongate strip of felt having the texture, feel and appearance of fine fur felt, the steps of preparing and thoroughly intermixing fur fibers and casein fibers to produce a blend; humidifying the blend; straightening the fibers of the blend into a thin web by a modified carding action; building up from the thin web a thick elongate bat on a support, maintaining the blend humid during the carding and bat forming; removing the elongate

bat from the support; and hardening and fulling the bat into a fabric by the wool felt process.

6. In the method of producing an elongate strip of felt having the texture, feel and appearance of fine fur felt, the steps of preparing and thoroughly intermixing fur fibers and synthetic fibers of the class consisting of casein and soybean fibers to produce a blend; humidifying the blend; straightening the fibers of the blend into a thin web by a modified carding action; building up from the thin web a thick elongate bat on a support, maintaining the blend humid during the carding and bat forming; removing the elongate bat from the support; and hardening and fulling the bat into a fabric by the 15 wool felt process.

7. In the method of producing yardage felt fabric having the texture, feel and appearance of fine fur felt, the steps of thoroughly intermixing fur fibers and an artificial feltable fiber of 20 the group consisting of center-seeking cotton, casein and soybean fibers and mixtures thereof

to form a blend thereof, humidifying the blend; straightening the fibers of the blend into a thin web by a modified carding action; superposing a plurality of the thin webs to build up a thick elongate bat; and felting the bat by the usual wool felt process into a fabric.

GEORGE M. RICKUS.

#### REFERENCES CITED

10 The following references are of record in the file of this patent:

#### UNITED STATES PATENTS

| Number    | Name          | Date          |
|-----------|---------------|---------------|
| 143,528   | Pollard       | Oct. 7, 1873  |
| 1,253,532 | Robinson      | Jan. 15, 1918 |
| 2,181,043 | Boeddinghaus  | Nov. 21, 1939 |
| 2,322,254 | Rickus et al. | June 22, 1943 |
| 2,322,255 | Rickus        | June 22, 1943 |
| 2,355,598 | Rickus et al. | Aug. 8, 1944  |
| 2,441,390 | Boeddinghaus  | May 11, 1948  |